

## UNITED STATES PATENT OFFICE

1,986,291

## MANUFACTURE OF ABSORBENT WATER-LAID WEBS OF FELTED FIBER

Milton O. Schur, Berlin, N. H., assignor to Brown Company, Berlin, N. H., a corporation of Maine

No Drawing. Application November 23, 1933,  
Serial No. 699,467

10 Claims. (Cl. 92—21)

This invention relates to the manufacture of porous and absorbent waterlaid webs of felted fiber on Fourdrinier or other paper-making machines from suitable aqueous fiber suspensions or so-called paper-making stocks. The objective of this invention is the economical production, more especially from cellulose fiber of the nature of chemical wood pulp, rag pulp, or the like, of webs or felts sufficiently porous and absorbent to lend themselves with facility to uniform impregnation with liquid or liquefied binders which can be dried, coagulated, congealed, or otherwise set or solidified in the impregnated sheet so as to render the sheet useful for various purposes in the arts, depending upon the qualities imparted thereto by the particular binder used as the impregnant. Inasmuch as the present invention devolves more particularly about the manufacture of the felt base, I shall dwell thereupon and indicate only in a general way the sort of impregnated product into which it may enter.

When the production of webs or felts of a porous and absorptive character is attempted on the usual paper-making machines, for instance, a Fourdrinier machine, difficulties are likely to arise. The seriousness of the difficulties met with varies, depending upon the particular paper-making stock delivered to the machine and the porosity and absorbency sought in the resulting webs or felts. In any event, however, one is faced with the problem of operating a paper-making machine having a dry end or drier section of given length and capacity so that it will be productive of webs or felts of the appropriate dryness at its rated capacity or at as great a capacity as possible. In order to get the rated capacity out of a given paper-making machine, it is necessary to dewater the web or felt as much as possible through the action of squeeze rolls at the wet end of the machine. Such practice, however, leads to webs or felts of excessive density or compactness with most kinds of paper-making stock; and this may be true even when the stock is comparatively free as, for instance, when it includes a large or preponderant proportion of substantially unhydrated wood pulp of high alpha cellulose content. The possibility of by-passing the squeeze rolls at the wet end of the paper-making machine is obviously to be avoided, if possible, since such practice requires either an expensive enlargement of the dry end of the machine or a sacrifice in the production of the machine. A greater steam consumption is inevitable as a

result of such practice, as is also the problem of running a weaker and soggier web without rupture or other damage through the machine.

I have found that in the fabrication of porous and absorptive webs, it is distinctly desirable to add to the paper-making stock at any stage of its transformation into webs or felts, but before drying, suitable surface-tension-reducing reagents, preferably water-soluble ones, as in the form of aqueous solutions of water-soluble soaps or aqueous solutions of water-miscible liquids of the nature of alcohol, acetone, etc. This desirability resides in the fact that when such agents are added to the stock and the web is dried in the presence of such agent, its density or compactness is markedly less than when such agent is omitted, and further that this fact holds true even when the web is dewatered by the action of squeeze rolls at the wet end of the machine to substantially the fullest extent possible before it is dried. The practice of the present invention hence makes possible the operation of a Fourdrinier or other typical paper-making machines substantially at their rated capacities and at the same time the production of webs or felts which, for many purposes, have the appropriate porosity and absorbency. It is my belief that the undesirably high density or compactness that the web acquires when manufactured in the ordinary way is due not only to the squeezing which the web receives but also to the contractile, i. e., shrinking forces, set up by the water as it evaporates from the web on the dryer. These contractile forces are believed to vary with the surface-tension of the water during the drying operation. By providing in the wet web an agent which reduces the action of surface-tension during the subsequent drying operation, shrinkage of the web and the accompanying reduction of porosity and absorbency therein can be reduced so as to conduce to webs of the desired character even when material squeezing pressure is exerted on the wet web by the squeeze rolls at the wet end of the machine and/or when the paper-making stock is unfavorable in the absence of a surface-tension-reducing reagent to webs of the desired character. Depending upon the pressure exerted on the wet web and the nature of the paper-making stock, it is possible by the practice of the present invention to produce webs of a wide variety of desirable compactnesses, wherefore, while the principles of the present invention are applicable to greatest economic advantage when the wet web is dewatered to a maximum content

5

10

15

20

25

30

35

40

45

50

55

before drying, they also obtain when less dewatering is so accomplished, for instance, even when no dewatering is so accomplished, as in all such cases, the dried web has surprisingly lower compactness than webs made similarly, that is, from similar paper-making stock and with a similar setting of the press rolls at the wet end of the machine but in the absence of a surface-tension-reducing agent during the drying of the webs.

I shall now give a typical example of procedure falling within the purview of my invention and designed to yield a felt such as is eminently suitable for bituminization into roofing and flooring products. A felt-making stock was prepared by mixing the following ingredients:—65% substantially unbeaten or unhydrated refined wood pulp; 8% beaten waste paper; 24% beaten rags; 3% raw potato starch; sufficient water to form a suspension for delivery to a Fourdrinier machine, say, a suspension of about 3/4% to 1% solids content.

The foregoing ingredients were first mixed in a beater engine under conditions to preserve the substantially unhydrated condition of the refined wood pulp, which was of the unbleached variety having an alpha cellulose content of about 94%. The thick aqueous mixture produced in the beater engine was then diluted with water to the consistency appropriate for felt-making on a Fourdrinier machine and was run off on such a machine. The wet web formed from the stock was carried by the usual carrier felt through the press rolls of the machine which was set to squeeze the web sufficiently hard to remove substantially all the extractable water therefrom and thereby permit the machine to be run at a high capacity. Between the press rolls, a 1% solution of ammonium oleate was sprayed onto the wet web and the rate of addition of such soap solution to the web was controlled so as to infuse about 0.8% to 1% of soap into the dried web. The web delivered from the dry end of the machine had a basis weight of 220 and a compactness of 44. A web made in exactly the same way, but which did not undergo soaping before the drying operation, had a compactness of 57; and this higher compactness was reflected in a harder and stiffer web. The difference in quality between the two webs was readily discernible by merely feeling them. Indeed, samples of the two webs were handed to a number of persons unskilled in the art and they invariably had no trouble whatever in picking out the web of the present invention as being distinctly softer and bulkier than the webs made as ordinarily.

It is, of course, possible to use aqueous solutions of various water-soluble soaps, such as the ammonium, sodium and potassium soaps of various fatty acids, such as stearic, palmitic and oleic, as the surface-tension-reducing reagents in accordance with my invention. Solutions may also be used containing other wetting-out agents, such as Turkey red oil, monopole oil, or other sulphonated oils, and a great variety of reagents are available in the comparatively recent commercial development of wetting-out agents comprised of sulphonated naphthalene, usually having side-chains, or sulphonated fatty alcohols. The solutions may be used at various concentrations, although dilute solutions of, say, about 0.5% to 2% strength are generally to be preferred, since they effect the required surface-tension-reducing action and the soap residue left

thereby in the dried web can be regulated so as to be extremely small, say, about 0.5% to 2%. When volatile liquids like alcohol and acetone serve as the surface-tension-reducing reagents, they are volatilized during the drying of the web with the result that the dried web is substantially devoid of such agents. The effect of the surface-tension-reducing reagent may be had by its addition to the paper-making stock at any time before the drying operation. Thus, the agent may be added to the bulk paper-making stock and/or to the wet web as it is passing over the suction boxes and/or, as already described, to the wet web as it is proceeding to or between the press rolls. Any of the waters containing the surface-tension-reducing reagent removed from the wet web at the wet end of the machine may be recovered for reuse in other stock. For instance, when the surface-tension-reducing reagent is added to the bulk paper-making stock, the machine may be operated with a closed white-water system so as to avoid loss of the agent. When a solution of such agent is added to the wet web at the suction boxes or at the squeeze rolls, the water containing such agent sucked or squeezed from the web may be recovered and used as the vehicle for making a fresh solution of such agent.

By adjusting the pressure on the squeeze rolls at the wet end of the machine, it is possible to practice my invention to produce webs or felts of a compactness ranging from about 20 to 55. The lowest compactness value represents that attainable when little or no squeezing of the web is done at the wet end of the machine and when the web is made from a suitable paper-making stock, say, one consisting substantially only of refined wood pulp having an alpha cellulose content of about 93 to 96% or higher and in a practically unhydrated condition. The highest compactness value represents that attainable when maximum squeezing of the web is done at the wet end of the machine and when the paper-making stock, like that given in the foregoing example, includes a substantial proportion of hydrated cellulose fibers and even binders such as starch. Within the foregoing range of compactness, the webs may be handled satisfactorily and can be impregnated quickly and uniformly into products of greatly variant utility. Webs at the lower end of the compactness range yield upon impregnation with rubber latices of suitable composition, and drying, mellow, pliant, artificial leathers such as can, after suitable finishing treatments, be used to good advantage in the uppers of shoes. Webs at the upper end of the compactness range can also be impregnated with rubber latex compositions and then dried to produce artificial leathers possessed of the stiffness requisite for such articles as welt inner soles. Webs in the intermediate zone or at the upper end of the compactness range can be bituminized most satisfactorily and to a high bitumen content to produce sheet material of value in the roofing and flooring industries. The foregoing are merely cited as being illustrative of only a few of many impregnated products in which the porous and absorbent webs or felts produced accordant with my invention may enter. I have hereinbefore referred to definite compactness values as being indicative of the density or compactness of webs fabricated according to my invention. These values of compactness are obtained by dividing the basis weight of the web in pounds by its thickness in

inches and multiplying by the factor  $10^{-2}$ . The expression "basis weight" to which I have also alluded as a definite value is known in paper-making circles as representing the weight in pounds of 480 sheets whose dimensions are 24x36 inches, this being equivalent to 2,880 square feet of sheet material. In other words, the compactness value really represents the weight of fiber per unit volume of sheet material.

I am aware of the fact that it has been proposed to introduce saponaceous or foam-generating materials into aqueous pulp suspensions for the purpose of causing a foam or lather therein and then depositing the fibers from the suspension into a distended mass of great voluminousness or bulkiness, which is dried in such distended condition. Such practice leads to a dry, bulky mass of fibers of such bulkiness as to disintegrate under light stresses and are unsatisfactory in many important instances for many practical impregnation treatments, especially continuous treatments. In the practice of my invention, even when I add water-soluble soaps to the bulk paper-making stock, I keep such stock substantially free from gas bubbles and foam so as to avoid improper felting of the fibers on account of interference by the gas bubbles or foam. I am also aware of the fact that it has been proposed to soap prefabricated waterleaf paper such as is to serve for toweling or similar purposes with aqueous soap solutions and then to redry the paper, the soap being thus added for the purpose of imparting the quality of emollients to the paper. A comparatively compact prefabricated paper web, that is, an ordinary web once dried, cannot, however, be restored to a materially less compact condition by the action of a soap solution thereupon, since the effect of compression and of shrinkage on the web once it has been dried cannot be undone to any great extent in this way. The fact of the matter is that a paper intended for toweling or similar use must have a compactness much greater than the webs produced according to my invention falling into a compactness range of about 20 to 55, since otherwise they would tend to disintegrate or pulp up in wet hands. Waterleaf paper toweling made from kraft pulp is said to contain a slight soap residue from the production of the kraft pulp, but this soap residue is of a resinous practically insoluble nature as can be readily appreciated from the fact that it is not dissolved and removed during the thorough washing operation which kraft pulp must necessarily undergo. The slight soap residue in kraft pulp hence does not function measurably as a surface-tension-reducing agent and, in any event, does not constitute a positive addition to the pulp but an occlusion that naturally and inevitably results from kraft pulp manufacture. It is hence impossible to realize the results of the present invention by depending upon the slight amount of resinous soap occluded on kraft pulp, so that should ordinary kraft pulp or kraft pulp refined to high alpha cellulose content be used in paper-making stock and the results of the present invention be desired from such stock, a solution of water-soluble soap or other surface-tension-reducing reagent must be used in the very same way as hereinbefore described. Nor are the results obtained by the practice of my invention possible of attainment when rosin soap or size is added to the paper-making furnish as is cus-

tomarily done in the manufacture of a great variety of papers, as in such case the soap or size is precipitated or insolubilized by a suitable reagent, usually alum, and hence does not exist as a surface-tension-lowering reagent during the drying of the paper web.

I have spoken about adding the surface-tension-reducing reagent to the paper-making stock at any stage of paper-making, but before drying. In saying this, I mean that this addition is effected before drying has proceeded to a stage where the action of surface-tension and shrinkage on the web has taken place to a material extent. In other words, the expression "but before drying", as used in the foregoing description and in the appended claims, is to be construed as comprehending the addition of surface-tension-reducing reagents part way down the drier, that is, while the web still contains sufficient water to be benefited by the surface-tension-reducing reagents, as such practice would be effective for the purposes of the present invention even though it would be comparatively less efficient.

So far as concerns certain subject-matter, the instant application is a continuation in part of my application Serial No. 495,785, filed November 14, 1930.

I claim:—

1. In the fabrication of a porous and absorbent waterlaid felt involving the formation of such felt from an aqueous suspension of a felt-making furnish containing cellulose fiber, those steps which comprise adding at any stage of felt fabrication, but before drying, to the water associated with the fiber a surface-tension-reducing agent while keeping such water substantially free from gas bubbles and foam, dewatering the felt to dryness, and controlling the composition of the furnish and/or the state of hydration of the cellulose fiber used in the furnish and/or the conditions under which the dewatering operation is performed so as to produce a felt of a compactness of about 20 to 55, said compactness being determined by dividing the basis weight of the felt in pounds by its thickness in inches and multiplying by the factor  $10^{-2}$ .

2. In the fabrication of a porous and absorbent waterlaid felt involving the formation of such felt from an aqueous suspension of a felt-making furnish containing cellulose fiber, those steps which comprise adding at any stage of felt fabrication, but before drying, to the water associated with the fiber a surface-tension-reducing agent while keeping such water substantially free from gas bubbles and foam, said surface-tension-reducing agent being selected from a class consisting of water-soluble soaps, wetting-out agents, alcohol, and acetone, dewatering the felt to dryness, and controlling the composition of the furnish and/or the state of hydration of the cellulose fiber used in the furnish and/or the conditions under which the dewatering operation is performed so as to produce a felt of a compactness of about 20 to 55, said compactness being determined by dividing the basis weight of the felt in pounds by its thickness in inches and multiplying by the factor  $10^{-2}$ .

3. In the fabrication of a porous and absorbent waterlaid felt involving the formation of such felt from an aqueous suspension of a felt-making furnish, those steps which comprise including cellulose fiber of high alpha cellulose content as an ingredient of the furnish, adding at any stage of felt fabrication, but before drying,

to the water associated with such fiber a water-soluble soap while keeping such water substantially free from gas bubbles and foam, dewatering the felt to dryness, and controlling the composition of the furnish and/or the state of hydration of the cellulose fiber used in the furnish and/or the conditions under which the dewatering operation is performed so as to produce a felt of a compactness of about 20 to 55, said compactness being determined by dividing the basis weight of the felt in pounds by its thickness in inches and multiplying by the factor  $10^{-2}$ .

4. In the fabrication of a porous and absorbent water-laid felt involving the formation of such felt from an aqueous suspension of a felt-making furnish containing cellulose fiber, those steps which comprise adding at any stage of felt fabrication, but before drying, to the water associated with the fiber ammonium oleate while keeping such water substantially free from gas bubbles and foam, dewatering the felt to dryness, and controlling the composition of the furnish and/or the state of hydration of the cellulose fiber used in the furnish and/or the conditions under which the dewatering operation is performed so as to produce a felt of a compactness of about 20 to 55, said compactness being determined by dividing the basis weight of the felt in pounds by its thickness in inches and multiplying by the factor  $10^{-2}$ .

5. In the fabrication of a porous and absorbent waterlaid felt involving the formation of such felt from an aqueous suspension of a felt-making furnish, those steps which comprise including as the preponderant fibrous ingredient of the felt-making furnish substantially unhydrated refined wood pulp of an alpha cellulose content of at least about 93%, adding to the wet felt at any stage of its fabrication, but before drying, a surface-tension-reducing agent, and drying the felt in the presence of such added agent, thereby producing a felt of compactness of about 20 to 55, said compactness being determined by dividing the basis weight of the felt in pounds by its thickness in inches and multiplying by the factor  $10^{-2}$ .

6. In the fabrication of a porous and absorbent waterlaid felt involving the formation of such felt from an aqueous suspension of a felt-making furnish, and the squeezing of the freshly formed wet felt before it is dried, those steps which comprise including as the preponderant fibrous ingredient of the felt-making furnish substantially unhydrated refined wood pulp of

an alpha cellulose content of at least about 93%, adding an aqueous soap solution to the freshly formed wet felt, squeezing the wet felt, and drying the squeezed felt in the presence of such added soap solution, thereby producing a felt of a compactness of about 20 to 55, said compactness being determined by dividing the basis weight of the felt in pounds by its thickness in inches and multiplying by the factor  $10^{-2}$ .

7. In the fabrication of a porous and absorbent waterlaid felt involving the formation of such felt from an aqueous suspension of a felt-making furnish containing cellulose fiber and the squeezing of the freshly formed felt before it is dried, those steps which comprise adding a surface-tension-lowering agent to the wet felt, squeezing the wet felt, drying the squeezed felt in the presence of such added agent, and controlling the composition of the furnish and/or the state of hydration of the cellulose fiber used in the furnish and/or the conditions under which the dewatering operation is performed so as to produce a felt of a compactness of about 20 to 55, said compactness being determined by dividing the basis weight of the felt in pounds by its thickness in inches and multiplying by the factor  $10^{-2}$ .

8. A porous and absorbent waterlaid fibrous felt falling within a range of compactness of about 20 to 55 and containing up to only about 2% of the residue of a solution of a water-soluble, surface-tension-lowering agent, based on the dry weight of the felt, said compactness being determined by dividing the basis weight of the felt in pounds by its thickness in inches and multiplying by the factor  $10^{-2}$ .

9. A porous and absorbent waterlaid fibrous felt falling within a range of compactness of about 20 to 55 and containing not more than about 0.5% to 2% of the residue of a solution of a water-soluble soap, based on the dry weight of the felt, said compactness being determined by dividing the basis weight of the felt in pounds by its thickness in inches and multiplying by the factor  $10^{-2}$ .

10. A porous and absorbent waterlaid fibrous felt falling within a range of compactness of about 20 to 55 and containing not more than about 0.5% to 2% of the residue of an aqueous solution of ammonium oleate, based on the dry weight of the felt, said compactness being determined by dividing the basis weight of the felt in pounds by its thickness in inches and multiplying by the factor  $10^{-2}$ .

MILTON O. SCHUR. 55